

## UNITED STATES PATENT OFFICE

2,600,995

## TUNGSTEN ALLOY

Jacob Kurtz, Teaneck, N. J., assignor, by mesne assignments, to Sylvania Electric Products, Inc., New York, N. Y., a corporation of Massachusetts

No Drawing. Application October 30, 1945,  
Serial No. 625,691.

7 Claims. (Cl. 75—22)

1

The present invention relates to sintered alloys of tungsten of good machinability, high density and hardness.

Tungsten is well known to be a very refractory metal in the sense that it has a melting point of about 3400° C. Such a refractory metal may be worked in the most economical manner by powder metallurgy methods, and such methods are generally employed in producing this metal for commercial uses. The tungsten powder is first shaped into ingot form in a mold under high pressure. It is then presintered in a hydrogen atmosphere at a temperature of 1000° C. so that the ingot can then be handled. The next step, accordingly, is to place the ingot in an electric circuit, also in a hydrogen atmosphere, and pass a current through it equivalent to about 90% of its fusing temperature, or about 2900° C., thus finally sintering it.

At this stage of working, the tungsten ingot is very strong, rather brittle and quite hard. Its density, however, must be further increased, and other desirable qualities must be given it. This is effected by swaging the ingot under heat. The rod so formed has a theoretical density of about 19.3 grams per cubic centimeter, and may be drawn down to very fine wires of a tensile strength far surpassing that of steel piano wire of equal diameter.

In many other respects, however, the pure hot swaged tungsten metal leaves much to be desired. It is very hard to machine; for instance, and consequently only the simplest shapes can be made from it, either by cutting off sections of a rod of circular cross-section, or by punching circular pellets from a flat sheet, both of which methods have been used in making electrical contact points for automobiles.

The uses of this very desirable metal can be increased to a very great extent if it can be made amenable to a greater degree of working that would make it possible to form it into shapes having a wider field of usefulness without greatly impairing its inherent natural qualities.

In application for patent of Kurtz and Williams, Serial No. 460,226, now Patent No. 2,491,866, issued December 20, 1949 there is disclosed an alloy consisting mainly of tungsten but having alloyed therewith small quantities of grain refining metal such as vanadium, and alloying, bonding and densifying metals such as manganese, iron, cobalt and nickel, and metal of the platinum family, and gold. This metal by sintering without swaging can be made with a density as high as or higher than that of pure hot swaged tungsten.

It is an object of the present invention to produce an alloy of this general type which has suitability for use for contact points and similar articles, and which, while it has somewhat less

2

density than metal disclosed in the Kurtz and Williams applications, nevertheless has a very high density without swaging, is quite hard and has good machinability. It may also be molded into a wide variety of shapes such as crucibles, disks, plates, and, in fact, it can be formed to any specifications.

It is a further object to produce an alloy that is basically tungsten, that possesses in large part the desirable properties of pure hot swaged tungsten, but which is capable of machining and shaping to a degree that is impossible with pure hot swaged tungsten. The alloy of the present invention is sintered at temperatures no higher than the range of rapid germination temperatures, but is comparable with pure hot swaged tungsten in density, and superior to it in machinability, and many other properties.

It has previously been pointed out that in the range of 1300°–1800° C., rapid crystallization of tungsten takes place and it is at these temperatures that the present alloy is sintered for a period sufficient to produce a large number of fine crystals. It is proposed in the method of the present invention not to exceed these temperatures greatly.

I have found that in powder metallurgy methods as applied to tungsten, the coherence and fineness of grain can be considerably promoted by adding to the basic tungsten metal powders certain other powdered metals having melting points within or slightly below the rapid crystallization range of the tungsten metal as hereinabove defined.

35 The metals to be added to the refractory metals are cobalt and platinum, and copper or silver or both.

The addition of cobalt increases the density and fineness of grain at temperatures within the range stated, but the addition of cobalt alone gives an extreme hardness to the ultimate alloy that makes it difficult to machine.

Platinum, as an addition to the tungsten metal, has much the same effect as cobalt in increasing density though not hardness. However, the cobalt and the platinum may be so combined as additions to the tungsten as to give high density, sufficient hardness for the desired purpose, and good machinability. The addition of cobalt and platinum should be very small for the best effects. For instance, an addition of 5% cobalt, or even much less, produces an alloy of very high density, about 17.7 grams per cubic centimeter if 0.5% platinum be added. With so much cobalt, however, the resultant alloy is very hard and, while machinable, is very difficult to machine. It has a hardness on the Rockwell A scale of about 76–76.

Within the ambit of this invention it is intended to include an alloy of tungsten, with co-

balt also, in an amount not exceeding 5% and a platinum group metal in an amount not exceeding 1% and an amount of silver and copper not exceeding 10% combined.

As examples of such alloys, the following will serve:

|               | A    | B    | C    |
|---------------|------|------|------|
| Cobalt.....   | 1.0  | 5.0  | 2.0  |
| Tungsten..... | 89.9 | 84.0 | 90.0 |
| Platinum..... | 0.1  | 1.0  | 1.0  |
| Copper.....   | 5.0  | 5.0  | 4.0  |
| Silver.....   | 4.0  | 5.0  | 3.0  |

The proportions given are by weight.

Alloy A has a density of 17.2. It has good machinability and a hardness on the Rockwell A scale of about 63. It is a metal suited for contact points and other uses, such as electrodes of any desired shape.

Alloy B has a density of 16.7. It has considerable hardness due to the somewhat large cobalt addition, but is machined easily.

Alloy C has a density of 17.8, a hardness on the Rockwell A scale of about 63, and good machinability.

The additions of copper and silver in combination with cobalt and platinum promote the densifying action and I find them to be beneficial in increasing the conductivity of the alloy and improving the machinability. The alloys of the invention may contain for best results from 84%–90% tungsten, from 1%–5% cobalt, from 1%–10% of copper-silver or both combined, and from 0.1%–1.0% of platinum.

The platinum may be added as powder but is so small in amount that it preferably should be added to the powdered metals as a solution of a water-soluble compound, such as chlorplatinic acid, in order to secure even distribution.

The powdered metals are impregnated with the chlorplatinic acid solution and dried in the air. They are then pressed in a mold and heated in a non-oxidizing atmosphere at a temperature of 1300° C. to 1800° C. for from one to three hours. After this heat treatment the metal shows a remarkable grain growth. The grain count shows not less than 2000 grains per square millimeter and may be as high as 20,000 grains per square millimeter.

The metals added to the tungsten have in each case a melting point within or below the temperature of rapid crystallization of the tungsten, namely, 1300° C. to 1800° C. Under the heat treatment given, a homogeneous alloy is formed with a minimum of voids and a density in the neighborhood of 17, a hardness of about 63 on the Rockwell A scale and good machinability. In general it may be stated that with the increase of the amount of cobalt, there is an increase in hardness, a property which is desirable in many instances, but if the addition of cobalt be too great, that is, much beyond 5%, the hardness increases to such an extent that machining is difficult if not impossible. The alloy formed from the constituents given is a homogeneous alloy characterized by very fine grain structure and a grain count of not less than 2,000 grains per square millimeter. If desired, after the sintering is completed, the sintered body may be subjected to a coining operation either at room temperature or at elevated temperatures.

Having thus described my invention, what I claim is:

1. A dense coherent tungsten alloy consisting

of 84% tungsten, 5% cobalt, 5% copper, 5% silver and 1% platinum, having a density of 16.7 grams per cubic centimeter and a grain count of not less than 2,000 grains per square millimeter and good machinability.

2. A dense coherent tungsten alloy consisting of 89.9% tungsten, 1% cobalt, 5% copper, 4% silver and 0.1% platinum, having a density of 17.2 grams per cubic centimeter and a grain count of not less than 2,000 grains per square millimeter and good machinability.

3. A dense coherent tungsten alloy consisting of 84% tungsten, 5% copper and 5% silver to which has been added as an addition cobalt and platinum in the relation of 5% cobalt to 1% platinum, having a density of 16.7 grams per cubic centimeter and a grain count of not less than 2000 grains per square millimeter and good machinability.

20 4. A dense coherent tungsten alloy consisting of 89.9% tungsten, 5% copper and 4% silver, and an addition of cobalt and platinum in the proportion of 1% cobalt to 0.1% platinum, having a density of 17.2 grams per cubic centimeter and 25 a grain count of not less than 2000 grains per square millimeter and good machinability.

5. A dense coherent tungsten alloy consisting of 90% tungsten, 4% copper and 3% silver and having an addition of cobalt and platinum in the 30 proportion of 2% cobalt to 1% platinum, said alloy having a density of 17.8 grams per cubic centimeter and a grain count of not less than 2000 grains per square millimeter and good machinability.

35 6. A dense coherent tungsten alloy consisting of 84% to 90% tungsten, 3% to 5% silver, 4% to 5% copper, 1% to 5% cobalt and .1 to 1% platinum, the alloy so formed having a density approximating 17 grams per cubic centimeter 40 and a grain count of not less than 2000 grains per square millimeter and good machinability.

7. A dense coherent tungsten alloy consisting of 84% to 90% tungsten, 1% to 10% copper-silver, 45 1% to 5% cobalt and .1 to 1% of platinum, the alloy so formed having a density approximating 17 grams per cubic centimeter and a grain count of not less than 2000 grains per square millimeter and good machinability.

JACOB KURTZ.

50

#### REFERENCES CITED

The following references are of record in the file of this patent:

#### UNITED STATES PATENTS

| Number       | Name          | Date          |
|--------------|---------------|---------------|
| 1,167,827    | Kaiser        | Jan. 11, 1916 |
| 1,346,192    | Gebauer       | July 13, 1920 |
| 1,447,797    | Adams         | Dec. 18, 1923 |
| 60 1,807,581 | Bates         | June 2, 1931  |
| 1,822,682    | Weiger        | Sept. 8, 1931 |
| 2,030,229    | Schwarzkopf   | Feb. 11, 1936 |
| 2,072,368    | Jedele        | Mar. 2, 1937  |
| 2,183,359    | Smithells     | Dec. 12, 1939 |
| 65 2,370,242 | Hensel et al. | Feb. 27, 1945 |
| 2,389,060    | Kurtz         | Nov. 13, 1945 |

#### FOREIGN PATENTS

| Number     | Country       | Date         |
|------------|---------------|--------------|
| 70 447,567 | Great Britain | May 21, 1936 |

#### OTHER REFERENCES

Hansen: Aufbau de Sweistofflegierungen, published by Edwards Brothers, Ann Arbor, Michigan 1936, pages 606-609, 1025 and 1026.